

# UNITED STATES PATENT OFFICE.

EDMUND R. BULLOCK, OF ROCHESTER, NEW YORK, ASSIGNOR TO EASTMAN KODAK COMPANY, OF ROCHESTER, NEW YORK, A CORPORATION OF NEW YORK.

## TONING PROCESS AND PRODUCT THEREOF.

1,286,890.

Specification of Letters Patent.

Patented Dec. 3, 1918.

No Drawing.

Application filed June 20, 1917. Serial No. 175,800.

To all whom it may concern:

Be it known that I, EDMUND R. BULLOCK, a subject of the King of Great Britain, residing in Rochester, in the county of Monroe and State of New York, have invented certain new and useful Improvements in Toning Processes and Products Thereof; and I do hereby declare the following to be a full, clear, and exact description of the same.

10 This invention relates to a toning process for photographic images and more particularly it concerns the toning of silver images and the improvement of the color of silver sulfid images. My invention also embraces 15 photographs which contain the toned image produced by my process.

One object of this invention is to provide a process which will be satisfactorily rapid, yet easily controlled and will yield pleasing, 20 stable, and readily duplicated tones. A further object is to obtain a photograph containing a toned image having the desirable qualities and color conferred upon it by my process.

25 It is well known to those skilled in the art that images of silver sulfid, which are customarily derived by bleaching a silver image in a bath containing potassium ferricyanid and potassium bromid and subsequently darkening the same in a bath of sodium sulfid, often have a tone which is unpleasantly yellow, particularly if the original silver image be weak or low in its principal densities and if the particle-size of the silver 30 halid be very small in the original emulsion. It is also known that a silver image may be converted into a derived image of silver selenid by treatment in a bath of selenium dissolved in sodium sulfid or sodium sulfite.

35 40 The resulting tone is a dark, cold purple, which is quite unsuited for many subjects. I have discovered, however, that I can produce an image, containing compounds of silver with both sulfur and selenium, which 45 has a pleasing tone that is redder and richer than the silver sulfid image and is warmer and redder than the silver selenid image. The principles of my method may be employed whether I start with a primary silver 50 image or with a silver sulfid image.

As a specific example of my process I shall describe its application to the toning of silver images suspended in suitable colloids such as gelatin, mounted on a paper, glass, 55 or film base. The primary silver image is

first treated in any usual or preferred bath or baths for the production of the secondary silver sulfid image. For instance, I may employ a bleaching bath of potassium ferricyanid and potassium bromid followed by a 60 bath of sodium sulfid, which is the socalled "redeveloping" method or I may employ the customary hypo-alum toning bath. After the sulfiding process, the print may be dried and subsequently treated, or the wet print 65 may be immediately treated in an aqueous solution containing two-thirds of one per cent. (3%) selenium and six and two-thirds per cent. (6 2/3%) of sodium sulfite. The color of the image gradually and steadily changes, 70 the final result being attained in a few minutes. Because of the known stability of a silver sulfid image, this action of the selenium bath is quite remarkable and unexpected. The alteration in tone is from the 75 yellowish hue of the sulfid to a rich reddish-brown effect and, since the alteration proceeds steadily, any intermediate tone may be obtained by withdrawing the silver image from the bath at the proper stage of the 80 operation and washing it. This elasticity in manipulation also permits of the ready duplication of tone, so that whenever a satisfactory effect has been obtained, it may be 85 repeated and the operator need not be embarrassed by making a set of prints in which the images are of varying hues, as is often the case in unmodified sulfid toning. The color of the final image is due to compounds 90 of silver, sulfur, and selenium.

The toning bath may, of course, be altered as regards the proportion of the several ingredients. Sodium bisulfite may be substituted, if desired, for the sodium sulfite. Furthermore, the corresponding potassium, ammonium, and magnesium salts, either singly or together, may be substituted for or combined with the sodium salts mentioned. The exact formulæ of all the active agents in my toning bath are not definitely known, 100 but it is certain that the bath contains salts of some acids containing sulfur and selenium several such acids being, selenosulfuric acid ( $H_2SSeO_3$ ), seleniumtrithionic acids ( $H_2S_2SeO_6$ ) and ( $H_2SSe_2O_6$ ) and selenium- 105 pentathionic acid ( $H_2S_4SeO_6$ ).

While it is generally not preferred, on account of its odor, I may form my toning bath by dissolving the selenium in a solution of sodium sulfid instead of sulfite.

Even where the ordinary sulfid toning methods are chiefly depended upon to modify the color of the original silver image, my process may be employed as a very useful auxiliary to save too-yellow images that would otherwise be thrown away. The manipulation is the same as when treating the secondary sulfid image hereinabove mentioned.

Having thus described my invention, what I claim and desire to secure by Letters Patent of the United States, is:

1. The toning process which comprises converting a primary silver image into a secondary silver sulfid image and treating the latter in a bath containing a salt of an acid which contains selenium.

2. The toning process which comprises converting a primary silver image into a secondary image containing silver sulfid

and treating the secondary image in a bath containing a salt of selenosulfuric acid.

3. The toning process which comprises treating a silver sulfid image in a bath containing a salt of an acid which contains selenium.

4. The toning process which comprises treating a silver sulfid image in a bath containing a salt of selenosulfuric acid.

5. A photograph comprising an image of a somewhat reddish tone including compounds of silver, sulfur, and selenium.

In testimony whereof, I have signed this specification in the presence of two witnesses this 6th day of June, 1917.

EDMUND R. BULLOCK.

Witnesses:

C. E. MARTIN,  
FRED H. GARDNER.